# EUROPEAN PATENT SPECIFICATION

(11) **EP 0 162 710 B1**
(45) Date of publication and mention of the grant of the patent: **09.08.1989**
(21) Application number: 85303595.4
(22) Date of filing: 22.05.1985
(51) Int. Cl.: C21D 8/12

(54) **Method for producing grain-oriented silicon steel sheets**
Verfahren zum Herstellen kornorientierter Siliziumstahlbleche
Procédé pour la production de tôle en acier au silicium à grain orienté

(30) Priority: 24.05.1984 JP 103696/84; 05.06.1984 JP 113790/84; 05.12.1984 JP 255807/84; 08.03.1985 JP 44940/85
(43) Date of publication of application: 27.11.1985
(73) Proprietor: KAWASAKI STEEL CORPORATION, Chuo-Ku, Kobe-Shi Hyogo-Ken (JP)
(72) Inventor: Iida, Yoshiaki c/o Research Laboratories, 1 Kawasaki-Cho Chiba City (JP); Iwamoto, Katsuo c/o Research Laboratories, 1 Kawasaki-Cho Chiba City (JP); Matoba, Isao c/o Research Laboratories, 1 Kawasaki-Cho Chiba City (JP)
(74) Representative: Overbury, Richard Douglas

(56) References cited:
- EP-A- 0 047 129
- DE-A- 2 351 141
- GB-A- 1 480 514
- US-A- 3 333 992
- US-A- 4 042 425
- US-A- 4 171 994
- PATENT ABSTRACTS OF JAPAN, vol. 8, no. 118 (C-226)[1555], 31st May 1984; & JP - A - 59 31823 (KAWASAKI) 21-02-1984
- PATENT ABSTRACTS OF JAPAN, vol. 7, no. 209 (C-186)[1354], 14th September 1983; & JP - A - 58 107 417 (KAWASAKI) 21-06-1983
- PATENT ABSTRACTS OF JAPAN, vol. 7, no. 273 (C-198)[1418], 6th December 1983; & JP - A - 58 151 423 (KAWASAKI) 08-09-1983
- CHEMICAL ABSTRACTS, vol. 85, no. 22, 29th November 1976, abstract no. 164766k, Columbus, Ohio, US; & JP - A - 51 78733 (KAWASAKI); & JP - B - 56 38652

## Description

The present invention relates to a method for producing grain-oriented silicon steel sheets, and particularly relates to a method for producing grain-oriented silicon steel sheets having low iron loss without lowering their magnetic induction.

Grain-orientated silicon steel sheets are required to have high magnetic induction and low iron loss. There have been proposed various methods for lowering the iron loss, for example, a method wherein a steel having a high Si content is used; a method wherein a product steel sheet having a small thickness is produced; a method wherein secondary recrystallization grains highly aligned to (110)[001] orientation, that is, to Goss orientation are developed; a method wherein secondary recrystallization grains having small size are developed; and the like. Methods for developing secondary recrystallization grains highly aligned to Goss orientation are known, for example, a method disclosed in Japanese Patent Application Publication No. 15,644/65, wherein an Al-containing silicon steel sheet is cold rolled at a high final reduction rate; a method disclosed in Japanese Patent Laid-open Specification No. 12,614/77 and the like, wherein a silicon steel having a very small B content is used; a method disclosed in Japanese Patent Application Publication No. 13,469/76, wherein an Sb-containing silicon steel sheet is subjected to a secondary recrystallization annealing at a low temperature; a method disclosed in Japanese Patent Application Publication No. 38, 652/81, wherein a cold rolled steel sheet having the final required gauge is annealed at a temperature within the range of 600-650°C for 0.5-10 minutes before the steel sheet is subjected to a decarburization annealing; a method disclosed in Japanese Patent Laid-open Specification No. 151,423/83, wherein a cold rolled steel sheet is heated in the heating stage of the decarburization annealing process at a rate of 100-400°C/min within a temperature range of 600-700°C in order that the recrystallization rate of the sheet steel be kept at about 50%; and the like.

According to these methods, the secondary recrystallized grains are surely and highly aligned to Goss orientation, and as a result a grain-oriented silicon steel sheet having high magnetic induction can be obtained. However the secondary recrystallized grains are always of coarse grain size, and the resulting grain-oriented silicon steel sheet still does not have a satisfactorily low iron loss.

Also, when it is intended to develop secondary recrystallization grains having a small grain size, not only crystal grains aligned to Goss orientation, but also crystal grains deviated from the Goss orientation grow as secondary recrystallization grains. Therefore, the resulting grain-oriented silicon steel sheet has low magnetic induction and high iron loss.

The object of the present invention is to obviate the drawbacks of the above described conventional techniques, and to provide a method whereby consistently stably grain oriented silicon steel sheets having excellent magnetic properties are produced, and wherein secondary recrystallization grains highly aligned to Goss orientation are developed and further the crystal grains are developed into a small size without forming into coarse grain size. Thereby the iron loss of the product steel sheet is lowered.

The inventors have made various investigations in order to solve the above described problems and found out that the above described object can be very effectively attained by the following methods, i.e. a method, wherein at least one member selected from the group consisting of elements of Ge, Sn, Pb, As, Bi and Zn and compounds containing these elements is applied to the surfaces of a finally cold rolled steel sheet before the decarburization annealing, or after the decarburization annealing and before the application of an annealing separator during the course of the production of a grain-oriented silicon steel sheet; a method wherein a step for subjecting a finally cold rolled steel sheet to a preliminary annealing at a temperature within the range of 500-700°C and a step for applying at least one member selected from the group consisting of elements of Ge, Sn, Pb, As, Bi and Zn and compounds containing these elements to the surfaces of a finally cold rolled steel sheet are carried out before the decarburization annealing of the finally cold rolled steel sheet during the course of the production of a grain-oriented silicon steel sheet; and a method wherein an annealing separator consisting mainly of MgO and further containing Bi or a compound containing Bi is coated onto the surfaces of a decarburized steel sheet before the secondary recrystallization annealing during the course of the production of a grain-oriented silicon steel sheet.

The present invention is based on the above described discoveries.

A first aspect of the present invention lies in a method of producing grain oriented silicon steel sheets, wherein a hot rolled silicon steel sheet containing at least one of S, Se and Te as an inhibitor to the growth of primary recrystallization grains is subject to at least one stage cold rolling. The finally cold rolled steel sheet is subjected to a decarburization annealing, and the decarburized steel sheet is coated with an annealing separator consisting mainly of MgO, and then subjected to a final annealing. The invention comprises applying uniformly at least one member selected from the group consisting of the elements Ge, Sn, Pb, As, Bi and Zn and compounds containing these elements to the surfaces of the finally cold rolled steel sheet before the decarburization annealing.

In a second aspect of the present invention at least one member selected from the group of elements Ge, Sn, Pb, As, Bi and Zn and compounds containing these elements is, advantageously, uniformly applied to the surfaces of the decarburized steel sheet, either additionally or exclusively, prior to the application of the annealing separator to the steel sheet surfaces.

In a third aspect of the present invention at least one member selected from the group consisting of the elements Ge, Sn, Pb, As, Bi and Zn and compounds containing these elements is uniformly applied to the surfaces of the finally cold rolled steel sheet and then the coated steel sheet is subjected to a preliminary annealing at a temperature within the range 500-700°C for 0.5 to 10 minutes prior to the decarburization annealing. The application of at least one member selected from the group consisting of the elements Ge, Sn, Pb, As, Bi and Zn and compounds containing these elements may also advantageously be made to the steel sheet, after the preliminary annealing, prior to the decarburization annealing.

A fourth aspect of the present invention lies in a method for producing grain oriented silicon steel sheets, wherein a hot rolled silicon steel sheet containing at least one of Si, Se and Te as an inhibitor for the growth of primary recrystallization grains is subjected to at least one stage cold rolling, the finally cold rolled steel sheet is subjected to a decarburization annealing, and the decarburized steel sheet is coated with an annealing separator consisting mainly of MgO, and then subjected to a final annealing wherein said annealing separator further contains at least one of Bi and compounds containing Bi.

For a better understanding of the invention, and to show how it may be carried out, reference will now be made, by way of example, to the accompanying drawings wherein:
Fig. 1 is a graph illustrating the relationship between the amount of Bi applied to silicon steel sheet surfaces before the decarburization annealing, and the magnetic induction, iron loss or average grain size of the resulting grain-oriented silicon steel sheet;
Fig. 2 is a graph similar to that of Fig. 1 and illustrating the relationship between the amount of Sn applied to silicon steel sheet surfaces before the decarburization annealing, and the magnetic induction, iron loss or average grain size of the resulting grain oriented silicon steel sheet;
Fig. 3 is a graph illustrating the relationship between the amount of Pb applied to silicon steel sheet surfaces after the decarburization annealing, and the magnetic induction, iron loss or average grain size of the resulting grain-oriented silicon steel sheet;
Fig. 4 is a graph illustrating the difference in the influence of the preliminary annealing temperature of a finally cold rolled silicon steel sheet upon the magnetic properties of the resulting grain-oriented silicon steel sheet between the method of the present invention, wherein a finally cold rolled steel sheet is coated with Zn and then subjected to the preliminary annealing, and a modified conventional method, wherein a finely cold rolled steel sheet is subjected to the preliminary annealing only, and further showing a comparison of the method of the present invention with the modified conventional method and a conventional method;
Fig. 5 is a graph illustrating the influence of the variant amount of Zn applied to the surfaces of a preliminarily annealed steel sheet before the decarburization annealing upon the magnetic properties of the resulting grain-oriented silicon steel sheet in the method of the present invention, and further showing a comparison of the method of the present invention with the modified conventional method and the conventional method;
Fig. 6 is a graph illustrating the relationship between the amount, calculated as Bi, of Bi₂(SO₄)₃ contained in an annealing separator, and the iron loss or magnetic induction of the resulting grain-oriented silicon steel sheet;
Fig. 7 is a graph illustrating the relationship between the concentration of Bi in a treating liquid for immersing a finally cold rolled steel sheet before the decarburization annealing, and the magnetic induction, iron loss or average grain size of the resulting grain-oriented silicon steel sheet; and
Fig. 8 is a graph illustrating the relationship between the immersing time of a finally cold rolled steel sheet, and the iron loss or average grain size of the resulting grain-oriented silicon steel sheet.

In the present invention, as the compounds containing Ge, _{'}Sn, Pb, As, Bi or Zn, the following compounds are preferably used;

Ge-containing compound:
GeO₂, GeC1₄ and the like

Sn-containing compound:
SnS, SnS0₄, Sn0₂, Na₂SnO₃, Sn(N0₃)₂ and the like

Pb-containing compound:
PbO_{z}, PbS, PbS0₄ and the like

As-containing compound:
As₂O₅, As_{z}0₃, As_{z}S₃, NaAsO₂ and the like

Bi-containing compound:
Bi₂(SO₄)_{3,} BiS, NaBi0₃, Bi_{z}0₃, Bi(N0₃)₂ and the like

Zn-containing compound:
ZnS, ZnS0₄, ZnO and the like

In the present invention, the above described elements and compounds containing these elements are applied to the surfaces of the finally cold rolled steel sheet before or after the steel sheet is subjected to the decarburization annealing. When the element or the compound is applied to the steel sheet surfaces before the decarburization annealing, it is advantageous that the element or the compound is applied to both surfaces of the steel sheet in an amount of at least 2 µg/m² calculated as element; and when the element or the compound is applied to the surfaces of the decarburized steel sheet, it is advantageous that the element or the compound is applied to both surfaces of the steel sheet in an amount of at least 10 µg/m² calculated as element.

When an annealing separator consisting mainly of MgO and further containing Bi or a Bi-containing compound is used, the amount of Bi or Bi-containing compound to be contained in the annealing separator is preferably about 0.1-5.0% calculated as Bi (in the specification, abstract of the disclosure and claims, "%" relating to amount means "% by weight" unless otherwise indicated).

The first aspect of the present invention will be explained referring to experimental data shown in Figs. 1 and 2.

A hot rolled silicon steel sheet having a thickness of 3.0 mm and having a composition containing C: 0.049%, Si: 3.2%, Mn: 0.06% and further containing Se: 0.025% and Sb: 0.050% was annealed at 1,000°C for 1 minute and then subjected to two stage cold rolling with an intermediate annealing at 950°C for 2 minutes to produce a cold rolled sheet having a final gauge of 0.30 mm. The finally cold rolled sheet was degreased, immersed in an aqueous dispersion of NaBi0₃, and then subjected to a decarburization annealing for 3 minutes in wet hydrogen kept at 830°C. The decarburized sheet was coated with an annealing separator consisting mainly of MgO, and then subjected to a final annealing at 1,200°C for 5 hours under hydrogen atmosphere. In the above described immersion treatment, the concentration of NaBi0₃, the temperature of the dispersion, and the immersing time were controlled so as to change variously the amount of Bi to be applied to the steel sheet surfaces. Further, during the final annealing, secondary recrystallization texture was fully developed within the temperature range of 820-900°C.

Fig. 1 shows the influence of the applied amount of Bi to the steel sheet surfaces upon the grain size and magnetic properties of the resulting grain-oriented silicon steel sheet.

It can be seen from Fig. 1 that, when at least 2 Ilg/m2 of Bi is applied to steel sheet surfaces before the decarburization annealing, the grain size of the product steel sheet becomes effectively small, the magnetic induction Bₗₒ thereof improves, and as the result the iron loss W_{17/50} thereof decreases considerably.

Similarly, a hog rolled silicon steel sheet having a thickness of 3.0 mm and having a composition containing C: 0.049%, Si: 3.2%, Mn: 0.06% and further containing inhibitors A-D shown in the following Table 1 was annealed at 1,000°C for 1 minute, and then subjected to two stage cold rolling with an intermediate annealing at 950°C for 2 minutes to produce a finally cold rolled sheet having a final gauge of 0.30 mm. The finally cold colled sheet, after degreasing, was immersed in an aqueous solution of SnS0₄, and then subjected to a decarburization annealing for 3 minutes in wet hydrogen kept at 830°C, and the decarburized steel sheet was coated with an annealing separator consisting mainly of MgO and then subjected to a final annealing at 1,200°C for 5 hours under hydrogen atmosphere.

In the above described immersion treatment in the aqueous SnS0₄ solution, the concentration of SnS0₄, the temperature of the solution and the immersing time were controlled so as to change variously the amount of Sn to be applied to the steel sheet surfaces. Further, during the final annealing, the secondary recrystallization texture was fully developed within the temperature range of 820―900°C.

Fig. 2 shows the influence of the amount of Sn applied to the steel sheet surfaces upon the grain size and magnetic properties in the resulting grain-oriented silicon steel sheet.

It can be seen from Fig. 2 that, when at least 2 pg/m² of Sn is applied to steel sheet surfaces before the decarburization annealing, the grain size in the product steel sheet becomes small, and the magnetic induction B₁₀ thereof improves, and as the result the iron loss W_{17/50} thereof decreases considerably.

The above described experiments explain the effect of the use of Bi- or Sn-containing compound as a surface treating agent. However, the inventors have made the same experiments as described above by using elements of Bi, Sn, Ge, Pb, As, and Zn and compounds containing Ge, Pb, As and Zn, and have examined the influence of these elements and compounds containing Ge, Pb, As and Zn, applied to the surfaces of the finally cold rolled steel sheet before the decarburization annealing upon the magnetic properties of the resulting grain-oriented silicon steel sheet, and ascertained that the same results as those shown in Figs. 1 and 2 are obtained.

The second aspect of the present invention will be explained referring to experimental data shown in Fig. 3.

A hot rolled silicon steel sheet having a thickness of 3.0 mm and having a composition containing C: 0.049%, Si: 3.2%, Mn: 0.06% and further containing Se: 0.025% and Sb: 0.050% was annealed at 1,000°C for 1 minute and then subjected to two stage cold rollings with an intermediate annealing at 950°C for 2 minutes to produce a finally cold rolled steel sheet having a final gauge of 0.3 mm. The finally cold rolled sheet was degreased, and then subjected to a decarburization annealing for 3 minutes in wet hydrogen kept at 830°C, and further immersed in an aqueous dispersion of Pb0₂. The immersion-treated steel sheet was coated with an annealing separator consisting mainly of MgO, and then subjected to a final annealing at 1,200°C for 5 hours under hydrogen atmosphere. In the immersion treatment, the concentration of Pb0₂, the temperature of the dispersion, and the immersing time were controlled so as to change variously the amount of Pb0₂ to be adhered to the steel sheet surfaces. Further, during the final annealing, secondary recrystallization texture was fully developed within the temperature range of 820-900°C.

Fig. 3 shows the influence of the amount of Pb applied to decarburized steel sheet surfaces upon the magnetic properties of the resulting grain-oriented silicon steel sheet.

It can be seen from Fig. 3 that, when at least 10 Ilg/m2 of Pb is applied to the decarburized steel sheet surfaces before the final annealing of the sheet, the crystal grain size of the product steel sheet becomes small, the magnetic induction B₁₀ thereof improves, and as the result the iron loss W_{17/50} thereof decreases considerably.

The inventors have made the same experiment as described above with respect to elements of Pb, Ge, Sb, As, Zn and Bi and compounds containing Ge, Sb, As, Zn and Bi, and ascertained that the same result as that shown in Fig. 3 is obtained.

One embodiment of the third aspect of the present invention will be explained hereinafter referring to experimental data shown in Fig. 4.

A hot rolled silicon steel sheet having a thickness of 2.5 mm and having a composition containing C: 0.049%, Si: 3.2%, Mn: 0.06% and further containing Se: 0.025% and Sb: 0.050% was annealed at 1,000°C for 1 minute and then subjected to two stage cold rollings with an intermediate annealing at 970°C for 2 minutes to produce a finally cold rolled sheet having a final gauge of 0.27 mm. The finally cold rolled sheet, after degreasing, was immersed for 10 seconds in an aqueous dispersion containing 100 mg/I of ZnO and kept at 30°C, and then squeezed by means of a pair of rubber rollers, and dried in an air bath kept at 200°C to adjust the amount of Zn to be applied to the steel sheet surfaces to 4.1 mg/m^{2.} The thus treated steel sheet was subjected to a preliminary annealing at a temperature within the range of 500-700⁰C for 2 minutes in dry nitrogen, and then subjected to a decarburization annealing for 3 minutes in wet hydrogen kept at 830°C. The decarburized steel sheet was coated with an annealing separator consisting mainly of MgO, and then subjected to a final annealing at 1,200°C for 5 hours under hydrogen atmosphere to produce a grain-oriented silicon steel sheet (this method of the third aspect of the present invention is indicated by the mark Φ in Fig. 4).

For comparison, the same hot rolled silicon steel sheet as described above was used, and a grain-oriented silicon steel sheet was produced in the same manner as described above, except that the finally cold rolled and degreased steel sheet was directly subjected to the decarburization annealing, carrying out neither the application of Zn nor the preliminary annealing (this method is a conventional method and is indicated by the mark 0 in Fig. 4).

Further, the same hot rolled silicon steel sheet as described above was used, and a grain-oriented silicon steel sheet was produced in the same manner as described above, except that the finally cold rolled and degreased steel sheet was subjected to the preliminary annealing without carrying out the application of Zn, and then subjected to the decarburization annealing (this method is modified conventional method and is indicated by the mark A in Fig. 4).

It can be seen from Fig. 4 that the modified conventional method (indicated by the mark A) is remarkably effective for improving the B₁₀ value of the resulting grain-oriented silicon steel sheet as compared with the conventional method (indicated by the mark O), but still has a drawback in that the resulting grain-oriented silicon steel sheet is rather high in the iron loss value as compared with the conventional method since the modified conventional method forms coarse secondary recrystallization structure having a remarkably large grain size. On the contary, according to the method of the third aspect of the present invention (indicated by the mark 8), the resulting grain-oriented silicon steel sheet does not have coarse crystal grains, but rather has small crystal grains, and as a result the grain-oriented silicon steel sheet has remarkably low iron loss value and further has remarkably high B₁₀ value.

This preliminary annealing is carried out at a temperature within the range of 500-700⁰C, preferably 500―650°C, for 0.5 to 10 minutes. The reason is as follows. The recrystallization begins generally at about 550°C, and proceeds rapidly as the temperature rises. A recrystallization texture for the preferred magnetic properties of the resulting grain-oriented silicon steel sheet can be obtained at a temperature of not higher than 650°C. In the preliminary annealing, when the annealing temperature is low, treatment for a longer time is effective for the annealing; and when the annealing temperature is high, treatment for a shorter time is effective for the annealing. However, a preliminary annealing for less than 0.5 minute or more than 10 minutes does not result in a satisfactory recrystallization texture, and the magnetic properties of the product steel sheet cannot thus be improved.

In the above described experiments, the effect of the use of a Zn-containing compound as a surface- treating agent has been explained. However, the inventors have made the same experiments as described above with respect to elements of Zn, Ge, Sn, Pb, As and Bi, and compounds containing Ge, Sn, Pb, As and Bi, and have ascertained that the same results as shown in Fig. 4 are obtained.

Further, another embodiment of the third aspect of the present invention will be explained by referring to experimental data shown in Fig. 5.

A hot rolled silicon steel sheet having a thickness of 2.2 mm and having the same composition as described above was annealed at 1,000°C for 1 minute, and then subjected to two stage cold rollings with an intermediate annealing at 970°C for 2 minutes to produce a finally cold rolled sheet having a final gauge of 0.23 mm. The finally cold rolled steel sheet, after degreasing, was subjected to a preliminary annealing wherein the steel sheet was heated at a heating rate of 100°C/min within the temperature range of 500-700°C, and then immersed in aqueous dispersion of ZnO such that the amount of ZnO to be applied to both surfaces of the steel sheet would be within the range of 10-³ mg/m²―10⁴ mg/m². The immersion-treated sheet was subjected to a decarburization annealing for 3 minutes in wet hydrogen kept at 830°C, then coated with an annealing separator consisting mainly of MgO, and then subjected to a final annealing at 1,200°C for 5 hours under hydrogen atmosphere to produce a grain-oriented silicon steel sheet (this method of the third aspect of the present invention is indicated by the mark A in Fig. 5).

For comparison, the same hot rolled silicon steel sheet as described above was used, and a grain-oriented silicon steel sheet was produced in the same manner as described above, except that the finally cold rolled and degreased steel sheet was directly subjected to the decarburization annealing, carrying out neither the preliminary annealing nor the application of Zn to the steel sheet surfaces (this method is a conventional method and is indicated by the mark 0 in Fig. 5).

Further, the same hot rolled silicon steel sheet as described above was used, and a grain-oriented silicon steel sheet was produced in the same manner as described above, except that the finally cold rolled and degreased steel sheet was subjected to the preliminary annealing and then to the decarburization annealing without carrying out the application of Zn to the steel sheet surfaces (this method is a modified conventional method and is indicated by the mark A in Fig. 5).

Fig. 5 shows the magnetic properties of the resulting products.

It can be seen from Fig. 5 that the product obtained by the modified conventional method (indicated by the mark A) has remarkably higher magnetic induction B₁₀ than that of the product by the conventional method (indicated by the mark 0), but does not have a satisfactorily low iron loss due to the development of coarse crystal grains. On the contrary, the product obtained by the method (indicated by the mark A) satisfying the conditions defined in the present invention has a remarkably low iron loss value due to the small crystal grain size in the product and further has remarkably high magnetic induction Bₗₒ.

In the above described experiments, the effect of the use of a Zn-containing compound as a surface- treating agent has been explained. However, the inventors have made the same experiments as described above with respect to elements of Zn, Ge, Sn, Pb, As and Bi, and compounds containing Ge, Sn, Pb, As and Bi, and have ascertained that the same results as shown in Fig. 5 are obtained.

The fourth aspect-of the present invention will be explained referring to experimental data shown in Fig. 6.

A hot rolled silicon steel sheet having a thickness of 2.0 mm and having a composition containing C: 0.049%, Si: 3.2%, Mn: 0.06% and further containing Se: 0.025% and Sb: 0.050% was annealed at 1,000°C for 1 minute and then subjected to two stage cold rolling with an intermediate annealing at 950°C for 2 minutes to produce a finally cold rolled sheet having a final gauge of 0.23 mm. The finally cold rolled sheet, after degreasing, was subjected to a decarburization annealing for 3 minutes in wet hydrogen kept at 830°C, then coated with an annealing separator consisting mainly of MgO, and further subjected to a final annealing at 1,200°C for 5 hours under hydrogen atmosphere to produce a grain-oriented silicon steel sheet. In the application of the annealing separator, a variant amount of Bi₂(SO₄)₃ was combined with the annealing separator consisting mainly of MgO. Further, during the final annealing, secondary recrystallization texture was fully developed within the temperature range of 820-900⁰C.

Fig. 6 illustrates the influence of the content of Bi₂(S0₄)₃ in the annealing separator upon the magnetic properties of the resulting grain-oriented silicon steel sheet. It can be seen from Fig. 6 that, when an annealing separator contains 0.1-5.0%, calculated as Bi, of Bi₂(S0₄)₃, the product steel sheet has satisfactorily high magnetic induction B₁₀ and low iron loss W_{17/50.} Bi-containing compounds other than the above described Bi₂(SO₄)₃ exhibited the same effect as that of Bi₂(SO₄)₃. When the content of a Bi-containing compound in an annealing separator was less than 0.1% calculated as Bi, the effect of the Bi-containing compound hardly appeared, and when the content exceeded 5%, secondary recrstallized grains in the product steel sheets were not uniformly oriented, and the product steel sheet was poor in magnetic properties and further was poor in surface appearance due to the formation of spot-like flaws.

The present invention will be explained in more detail by consideration of the following production steps.

It is desirable that the steel should contain Si: 2.5-4.0%, C:0.02-0.06% and Mn: 0.02-0.20% and further contain at least one of S: 0.005-0.05%, Se: 0.005-0.05% and Te: 0.003-0.05%. Si is used for obtaining satisfactorily low iron loss without sacrificing the yield in the cold rolling, C is used for forming fine crystal grains in the steps carried out after hot rolling, and other ingredients are used for inhibiting effectively the growth of primary recrystallization grains. It is desirable that the initial silicon steel contains the above described ingredients in the above described range. However, even when the amounts are outside of the above described ranges, the ingredients still have an appreciable effect.

The initial silicon steel to be used in the present invention has a composition consisting of the above described ingredients and the remainder being substantially Fe and incidental impurities. However, the steel may occasionally contain grain boundary seggregation elements, such as Sb, As, Bi, Sn, Pb and the like, alone or in admixture in order to improve the effect of the inhibitors. The addition of the grain boundary segregation element does not have any adverse influence upon the effect of the present invention.

The invention is not affected by the steel making or hot rolling methods employed, hence these processes may be carried out according to commonly known methods.

The annealing of a hot rolled sheet and the intermediate annealing in the cold rolling step are occasionally carried out at a temperature within the range of 750-1,000°C for a period of from 10 seconds to 10 minutes.

The hot rolled sheet, after being occasionally annealed, is subjected to at least one stage cold rolling to produce a finaly cold rolled sheet having the final desired gauge. The finally cold rolled sheet is degreased by a commonly known method, and then at least one member selected from the group consisting of elements of Ge, Sn, Pb, As, Bi and Zn and compounds containing these elements is applied to the surfaces of the steel sheet. The method for applying the element or the element-containing compounds to the steel sheet surfaces can be any of immersion, spraying, application, electrodeposition, dropping, transfer printing and the like.

The amount of the element orthe element-containing compound to be applied to the surfaces of a steel sheet should be at least 2 pg/M2 calculated as element. It is preferable to apply the element or the element-containing compound to both surfaces of a steel sheet. However, it is not always necessary to apply the element or the element-containing compound to both surfaces of a steel sheet, and even when the element or`the element-containing compound is applied to only one surface of a steel sheet, the effect of the element appears. When the element or the element-containing compound is applied to one surface of a steel sheet, it is also necessary that the amount of element applied to one surface of the steel sheet is at least 2 pg/m² in order to produce a product steel sheet having excellent magnetic properties.

The above treated steel sheet is subjected to a decarburization annealing at a temperature of 700―900°C under an atmosphere containing hydrogen and steam until the C content in the steel sheet becomes about 0.003% or less.

In the third aspect of the present invention, prior to the above described decarburization annealing, the finally cold rolled and degreased steel sheet is subjected to a preliminary annealing such that the steel sheet is kept to a constant temperature within the range of 500-700⁰C for 0.5-10 minutes or its heated within the temperature range of 500―700°C at a heating rate of 50°C/min-400°C/min. This preliminary annealing is effective in improving the primary recrystallization texture.

The preliminary annealing may be carried out before the above described application of the element or the application treatment may be carried out before and after the preliminary annealing.

According to the second aspect of the present invention, the finally cold rolled and degreased steel sheet is directly subjected to a decarburization annealing at a temperature of 700-900⁰C under an atmosphere containing hydrogen steam until the C content in the steel sheet becomes about 0.003% or less, without carrying out the application of the element or a combination of the application of the element and the preliminary annealing. Then, at least one member selected from the group consisting of elements of Ge, Sn, Pb, As, Bi and Zn and compounds containing these elements is applied to the surfaces of the steel sheet. The method for applying the element or the element-containing compound to the steel sheet surfaces can be any of immersion, spraying, application, electrodeposition, dropping, transfer printing, and the like.

When the element or the compound containing the element is applied to the decarburized steel sheet, the amount of the element or the compound containing the element to be applied to the surfaces of the steel sheet is at least 10 pg/m² calculated as element. When the amount is less than 10 pg/m², the magnetic properties of the resulting grain-oriented silicon steel sheet are not satisfactorily improved. In the present invention, it is not always necessary to apply the element or the element-containing compound to both surfaces of a steel sheet, and even when the element or the element-containing compound is applied to only one surface of a steel sheet, the effect of the element appears. When the element or the element-containing compound is applied to one surface of a steel sheet, it is also necesssary that the amount of element applied to one surface of the steel sheet is at least 10 µg/m² in order to produce a product steel sheet having excellent magnetic properties.

When the finally cold rolled and degreased steel sheet is directly subjected to the decarburization annealing without carrying out the application of the element or a combination of the application of the element and the preliminary annealing, it is necessary to carry out the above described application of the element after the decarburization annealing. However, when the finally cold rolled and degreased steel sheet has been subjected to the application of the element or a combination of the application of the element and the preliminary annealing before the decarburization annealing, the decarburized steel sheet may be occasionally subjected to the application of element.

The essential feature of the first aspect of the present invention lies in that the application of the element or a combination of the application of the element and the preliminary annealing is carried out during a process wherein the finally cold rolled and degreased steel sheet is subjected to a decarburization annealing and then coated with an annealing separator consisting mainly of MgO in a conventional method.

In the first and second aspects of the present invention, the final cold rolling, the application of the element, and the decarburization annealing can be carried out according to the following treatment orders.

(1) final cold rolling-application treatment-decarburization annealing,
(2) final cold rolling-decarburization annealing-application treatment, and
(3) final cold rolling-application treatment-decarburization-application treatment.

Further, the final cold rolling, the application treatment of element, the preliminary annealing and the decarburization annealing in the third aspect of the present invention can be carried out according to the following treatment orders.

(4) final cold rolling-application treatment-preliminary annealing-decarburization annealing,
(5) final cold rolling-preliminary annealing-application treatment-decarburization annealing,
(6) final cold rolling-preliminary annealing-decarburization annealing-application treatment,
(7) final cold rolling-application treatment-preliminary annealing-application treatment-decarburization annealing,
(8) final cold rolling-application treatment-preliminary annealing-decarburization annealing-application treatment,
(9) final cold rolling-preliminary annealing-application treatment-decarburization annealing-application treatment, and
(10) final cold rolling-application treatment-preliminary annealing-application treatment-decarburization annealing-application treatment.

Of course, in the present invention, among the above described tratment orders, a proper treatment order must be selected depending upon the magnetic properties of the desired product.

The inventors have made an investigation with respect to the preferable treatment conditions for the immersion method for applying the element to the steel sheet surfaces. The results of the investigation will be explained hereinafter referring to Figs. 7 and 8.

A hot rolled silicon steel sheet having a thickness of 3.0 mm and having a composition containing C: 0.049%, Si: 3.2%, Mn: 0.06% and further containing inhibitors shown in the above described Table 1 was annealed at 1,000°C for 1 minute, and then subjected to two stage cold rolling with an intermediate annealing at 950°C for 2 minutes to produce a finally cold rolled sheet having a final gauge of 0.30 mm. The finally cold rolled sheet, after degreasing, was immersed in an aqueous dispersion containing NaBi0₃ powder dispersed therein, passed through a pair of squeeze rollers and then dried. The above treated steel sheet was subjected to a decarburization annealing at 830°C for 3 minutes in wet hydrogen, and the decarburized steel sheet was coated with an annealing separator consisting mainly of MgO, and then subjected to a final annealing at 1,200°C for 5 hours. In the above described immersion treatment in the NaBi0₃ dispersion, the concentration of Bi, the temperature of the dispersion, and the immersing time were controlled so as to change variously the amount of Bi to be applied to the steel sheet surfaces. Further, during the final annealing, secondary recrystallization texture was fully developed at a temperature within the range of 820-900⁰C.

Fig. 7 illustrates relationship between the concentration of Bi in the aqueous NaBi0₃ dispersion, and the magnetic properties of the resulting grain-oriented silicon steel sheet (final gauge: 0.30 mm).

It can be seen from Fig. 7 that, when a finally cold rolled and degreased steel sheet is immersed in an aqueous NaBi0₃ dispersion having a Bi concentration of at least 10 mg/l prior to the decarburization annealing, the resulting grain-oriented silicon steel sheet has small grain size, high magnetic induction and further significantly low iron loss, these being independent of the kind of inhibitors.

It has been ascertained from experiments that, even when an application method by means of a spray or fluted roll is used in place of the immersion method, substantially the same effect as described above can be obtained.

Fig. 8 illustrates relationship between the immersing time of a finally cold rolled and degreased steel sheet in an aqueous NaBi0₃ dispersion having a Bi concentration of 208 mg/I, and the grain size and iron loss value of the resulting grain-oriented silicon steel sheet (final gauge: 0.23 mm).

It can be seen from Fig. 8 that the iron loss value and grain size of the product steel sheet containing any kind of inhibitors are not substantially influenced by the immersing time, and even an immersion treatment of a short time of about 1 second is effective for attaining the object of the present invention.

Further, it has been ascertained that, even when an application method by means of a spray or fluted roll is used in place of the immersion method, substantially the same effect as described above can be obtained.

Accordingly, it is important in the immersion method that a finally cold rolled and degreased steel sheet is immersed for at least 1 second in an aqueous dispersion containing a given element in a concentration of at least 10 mg/I. After the immersion treatment, the immersed steel sheet is passed occasionally through a pair of squeeze rollers and then dried. By this squeezing treatment, the amount of an element to be adhered to the steel sheet surfaces can easily be controlled. The drying is a very important treatment in order to give satisfactorily high rust resistance to the resulting grain-oriented silicon steel sheet and further to give an excellent appearance to the coating film formed on the steel sheet surfaces.

When an aqueous dispersion is used as a treating liquid, it is advantageous that the dispersion is formed into a sol or a colloidal dispersion or is fully stirred by means of a propeller or an ultrasonic wave in order to keep the concentration constant and to apply the element uniformly to the steel sheet surfaces.

After the finally cold rolled and degreased steel sheet is subjected to the above described application treatment of element and the decarburization annealing (in the first and second aspects of this invention), or after the finally cold rolled and degreased steel sheet is subjected to the above described application treatment of element, preliminary annealing and decarburization annealing (in the third aspect of this invention), the steel sheet is coated with an annealing separator consisting mainly of MgO.

According to the fourth aspect of the present invention, a finally cold rolled and degreased steel sheet is directly subjected to the decarburization annealing without carrying out the above described application treatment of element or a combination of the application treatment of element and the preliminary annealing, and an annealing separator consisting mainly of MgO and containing 0.1-5.0% of Bi or a Bi-containing compound is applied to the decarburized steel sheet.

Of course, the annealing separator consisting mainly of MgO and containing 0.1-5.0% of Bi or a Bi-containing compound may be coated onto a decarburized steel sheet, which has already been subjected to the application of element or a combination of the application of element and the preliminary annealing in the first, second or third aspect of the present invention.

The steel sheet coated with the above described annealing separator was subjected to a final annealing comprising a recrystallization annealing at a temperature within the range of 800-1,000°C and a purification annealing at a temperature within the range of 1,100-1,250°C under hydrogen atmosphere subsequent to the recrystallization annealing.

After removal of the annealing separator, the finaly annealed steel sheet was applied with a tension coating, and then subjected to a flattening annealing at a temperature within the range of 700-900°C.

Japanese Patent Application Publication No. 48;567/81 discloses a technique, wherein a compound containing any one of Al, Sn, As, Pb, Sb, Bi, Se and Te is applied to the surfaces of a cold rolled low-carbon aluminum killed steel sheet in an amount of at least 2 g/m² before the annealing of the steel sheet under a nitrogen-containing atmosphere, in order to prevent the nitriding of the steel sheet during the annealing. Further, this Japanese patent application publication discloses that the use of the above described element is also effective for preventing the deterioration of the electromagnetic properties of a silicon steel sheet due to its nitriding. On the contrary, according to the present invention, the magnetic properties of a silicon steel sheet can be remarkably improved by applying a very small amount of only several pg/_{M}² of element to its surface as illustrated in Figs. 1-3, and further the magnetic properties of silicon steel sheet can be remakarbly improved even by an annealing under an atmosphere not containing N₂, that is, an annealing under H₂ or Ar atmosphere as illustrated in the following Examples 1, 2, 3, 4, 5, 7, 9, 10 and 14. Accordingly, in the present invention, the magnetic properties of silicon steel are improved by preventing its nitriding, but are improved by giving to the steel a property entirely different from the prevention of nitriding. That is, the present invention has been accomplished based on a technical idea entirely different from that disclosed in the above described Japanese Patent Application Publication No. 48,567/81.

The following examples are given for the purpose of illustration of this invention and are not intended as limitations thereof.

### Example 1

A hot rolled sheet having a thickness of 3 mm and having a composition containing C: 0.052%, Si: 3.36%, Mn: 0.065%, Se: 0.025% and Sb: 0.031 % was cold rolled into a thickness of 0.80 mm, and the first cold rolled sheet was intermediately annealed at 950°C for 1 minute and then secondly cold rolled into a final gauge of 0.30 mm. The finally cold rolled sheet, after degreasing, was immersed for 2 seconds in an aqueous solution contaioning 160 mg/l of ZnS0₄ and kept at 30°C, and then passed through a rubber a pair of squeeze rollers and then dried. The amount of Zn adhered to the dried steel sheet was 15 mg/m². Then, the above treated steel sheet was subjected to a decarburization annealing for 3 minutes in wet hydrogen kept at 830°C, and the decarburized sheet was coated with an MgO slurry. The coated sheet was dried and then subjected to a final annealing at 850°C for 50 hours and successively at 1,200°C for 10 hours under H₂ atmosphere.

The following Table 2 shows the magnetic properties and grain size of the resulting grain-oriented silicon steel sheet. For comparison, a grain-oriented silicon steel sheet was produced according to a conventional method, wherein the finally cold rolled and degreased steel sheet was not treated with the aqueous ZnS0₄ solution but was directly subjected to the decarburization annealing. The magnetic properties and grain size of the product steel sheet are also shown in Table 2.

It can be seen from Table 2 that, when Zn is applied to the steel sheet surfaces before the decarburization annealing, the product steel sheet has small grain size, high magnetic induction and further significantly low iron loss.

### Example 2

A hot rolled sheet having a thickness of 2 mm and having a composition containing C: 0.040%, Si: 3.05%, Mn: 0.08%, S: 0.021 % and Te: 0.005% was cold rolled into a thickness of 0.60 mm, and the first cold rolled sheet was intermediately annealed at 900°C for 1 minute and then secondly cold rolled into a final gauge of 0.23 mm. The finally cold rolled sheet, after degreasing, was immersed for 5 seconds in an aqueous dispersion containing 1 g/t of finely divided GeO₂ and kept at 80°C, and then dried. In this immersion treatment, GeO₂ was applied to the surfaces of the steel sheet in an amount of 1 mg/m². The above treated steel sheet was subjected to a decarburization annealing in wet hydrogen kept at 830°C, and the decarburized sheet was coated with an MgO slurry. The coated sheet was dried and then subjected to a final annealing at 880°C for 20 hours under an Ar atmosphere and successively at 1,200°C for 10 hours under an H₂ atmosphere.

The following Table 3 shows the magnetic properties and grain size of the resulting grain-oriented silicon steel sheet together with those of a comparative grain-oriented silicon steel sheet produced by a conventional method.

It can be seen from Table 3 that, when a Ge-containing compound is applied to the-steel sheet surfaces before the decarburization annealing, the product steel sheet has small grain size, high magnetic induction and further significantly low iron loss.

### Example 3

A hot rolled sheet having a thickness of 2.0 mm and having a composition containing C: 0.048%, Si: 3.4%, Mn: 0.07%, Se: 0.02% and Sb: 0.03% was cold rolled into a final gauge of 0.60 mm. After degreasing, the finally cold rolled sheet was immersed for 1 minute in an aqueous dispersion containing 300 mg/I of PbS0₄ and kept at 80°C, and then passed through a pair of rubber squeeze rollers. The squeezed sheet was dried in an air bath kept at 150°C. The amount of PbO applied to both surfaces of the dried steel sheet was 1 mg/m². Then, the above treated steel sheet was subjected to a decarburization annealing at 840°C for 3 minutes under an atmosphere consisting of 50% by volume of H₂ and the remainder being N₂ and having a dew point of 60°C, and then applied with an MgO slurry, and further subjected to a final annealing at 880°C for 30 hours under an H₂ atmosphere and successively at 1,200°C for 10 hours under an H₂ atmosphere.

The following Table 4 shows the magnetic properties and grain size of the product steel sheet together with those of a comparative product steel sheet produced without the adhesion of Pb to the steel sheet surfaces according to the conventional method.

It can be seen from Table 4 that, when the finally cold rolled sheet is treated with a Pb-containing dispersion, the product steel sheet has very small crystal grain size and significantly low iron loss.

### Example 4

A hot rolled sheet having a thickness of 3 mm and having a composition containing C: 0.051 %, Si: 3.34%, Mn: 0.067%, S: 0.027% and Sb: 0.032% was cold rolled into a thickness of 0.80 mm, and the first cold rolled sheet was intermediately annealed at 950°C for 1 minute and then secondly cold rolled into a final gauge of 0.3 mm. After degreasing, the finally cold rolled sheet was immersed for 3 seconds in an aqueous dispersion containing 130 mg/I (75 mg/l calculated as As) of NaAs0₂ and kept at 30°C, passed through a pair of rubber squeeze rollers and then dried. The above treated steel sheet was subjected to a decarburization annealing at 830°C for 3 minutes in wet hydrogen, and the decarburized sheet was applied with an MgO slurry. After drying, the applied sheet was subjected to a final annealing at 850°C for 50 hours and successively at 1,200°C for 10 hours under an H₂ atmosphere.

The following Table 5 shows the magnetic properties and grain size of the resulting product steel sheet together with those of a comparative product steel sheet produced by a conventional method.

It can be seen from Table 5, that when As is applied to the steel sheet surfaces before the decarburization annealing, the resulting product steel sheet has small grain size, high magnetic induction and low iron loss, and the application of As to the steel sheet surfaces is very effective.

### Example 5

A hot rolled sheet having a thickness of 3 mm and having a composition containing C: 0.040%, Si: 3.22%, Mn: 0.089%, Se: 0.028% and Sb: 0.027% was annealed at 1,000°C for 1 minute, and then pickled. The pickled sheet was cold rolled into a thickness of 0.87 mm, and the first cold rolled sheet was intermediately annealed at 980°C for 1 minute and then secondly cold rolled into a final gauge of 0.30 mm. After degreasing, the finally cold rolled sheet was immersed for 15 seconds in an aqueous dispersion containing 800 mg/I of Bi₂0₃ and kept at 30°C, and then passed through a pair of rubber squeeze rollers, and further dried in an air bath kept at 150°C. The amount of Bi applied to the steel sheet surfaces was 4.9 mg/ m^{2.} The above treated steel sheet was subjected to a prelimary annealing at 600°C for 1 minute, and then to a decarburization annealing at 830°C for 3 minutes under an atmosphere consisting of 50% by volume of H₂ and the remainder being N₂ and having a dew point of 60°C. The decarburized steel sheet was coated with an MgO slurry, and then subjected to a final annealing at 860°C for 35 hours under an Ar atmosphere and successively at 1,200°C for 10 hours under an H₂ atmosphere.

The following Table 6 shows the magnetic properties of the resulting grain-oriented silicon steel sheet together with those of a comparative grain-oriented silicon steel sheet produced by a conventional method.

It can be seen from Table 6 that, when a Bi salt is applied to a finally cold rolled and degreased sheet before its decarburization annealing and further a preliminary annealing is carried out at 600°C for 1. minute during the course of heating for a decarburization annealing according to present invention, the resulting product steel sheet has remarkably low iron loss value and high B₁₀ value.

### Example 6

A hot rolled sheet having a thickness of 2.2 mm and having a composition containing C: 0.049%, Si: 3.38%, Mn: 0.088%, S: 0.027% and Sb: 0.023% was annealed at 950°C for 1 minute, and then pickled. The pickled sheet was cold rolled into a thickness of 0.58 mm, and the first cold rolled sheet was intermediately annealed at 980°C for 1.5 minutes and then secondly cold rolled into a final gauge of 0.23 mm. After degreasing, the finally cold rolled sheet was subjected to a preliminary annealing at 550°C for 4 minutes, and the preliminarily annealed sheet was immersed for 10 seconds in an aqueous dispersion containing 100 mg/I of SnO₂ and kept at 50°C, and then passed through a pair of rubber squeeze rollers, and further dried in an air bath kept at 200°C. The amount of Sn applied to both surfaces of the steel sheet was 0.96 mg/ m^{2.} The above treated steel sheet was subjected to a decarburization annealing at 840°C for 3 minutes under an atmosphere consisting of 55% by volume of H₂ and the remainder being N₂ and having a dew point of 55°C. The decarburized steel sheet was coated with an MgO slurry, and then subjected to a final annealing at 870°C for 25 hours under an N₂ atmosphere and successively at 1,200°C for 10 hours under an H₂ atmosphere.

The following Table 7 shows the magnetic properties of the resulting grain-oriented silicon steel sheet together with those of a comparative grain-oriented silicon steel sheet produced by a conventional method.

It can be seen from Table 7 that the product steel sheet of the present invention has a remarkably lower' iron loss value and higher B₁₀ value than those of the comparative product steel sheet.

### Example 7

A hot rolled sheet having a thickness of 2 mm and having a composition containing C: 0.041%, Si: 3.24%, Mn: 0.089%, S: 0.027% and Te: 0.005% was annealed at 970°C for 1 minute, and then pickled. The pickled sheet was cold rolled into a thickness of 0.50 mm, and the first cold rolled sheet was intermediately annealed at 980°C for 1 minute and then secondly cold rolled into a final gauge of 0.20 mm. After degreasing, the finally cold rolled sheet was immersed for 20 seconds in an aqueous dispersion containing 1.5 g/I of PbS0₄ and kept at 80°C, and then passed through a pair of rubber squeeze rollers, and further dried in an air bath kept at 200°C. The amount of Pb applied to both surfaces of the steel sheet was 1.25 mg/ m². The above treated steel sheet was subjected to a preliminary annealing by heating the steel sheet at a heating rate of 80°C/min. within the temperature range of 500-700°C under an atmosphere consisting of 55% by volume of H₂ and the remainder beiong N₂ and having a dew point of 60°C, and successively subjected to a decarburization annealing at 835°C for 3 minutes under the same atmosphere as described above. The decarburized steel sheet was coated with an MgO slurry, and then subjected to a final annealing at 860°C for 35 hours under an Ar atmosphere and successively at 1,200°C for 10 hours under an H₂ atmosphere.

The following Table 8 shows the magnetic properties of the resulting product steel sheet together with those of a comparative product steel sheet produced by a conventional method.

### Example 8

A hot rolled sheet having a thickness of 2.5 mm and having a composition containing C: 0.047%, Si: 3.35%, Mn: 0.090% and Se: 0.024% was annealed at 950°C for 2 minutes, and then pickled. The pickled sheet was cold rolled into a thickness of 0.71 mm, and the first cold rolled sheet was intermediately annealed at 980°C for 1 minute and then secondly cold rolled into a final gauge of 0.27 mm. After degreasing, the finally cold rolled sheet was immersed for 11 seconds in an aqueous dispersion containing 50 mg/l of NaAs0₂ and kept at 25°C and then passed through a pair of rubber squeeze rollers, and further dried in an air bath kept at 150°C. The amount of As applied to both surfaces of the steel sheet was 150 pg/m². The above treated steel sheet was subjected to a preliminary annealing by heating the steel sheet at a heating rate of 50°C/min within the temperature range of 500-700°C under an atmosphere consisting of 53% by volume of H₂ and the remainder being N₂ and having a dew point of 57°C, and successively subjected to a decarburization annealing at 830°C for 3 minutes under the same atmosphere as described above. The decarburized steel sheet was applied with an MgO slurry, and then subjected to a final annealing at 865°C for 40 hours under an N₂ atmosphere and successively at 1,200°C for 10 hours under an H₂ atmosphere.

The following Table 9 shows the magnetic properties of the product steel sheet of the present invention together with a comparative product steel sheet produced by a conventional method. It can be seen from Table 9 that the product steel sheet of the present invention has remarkably excellent magnetic properties as compared with those of the comparative product steel sheet.

### Example 9

A hot rolled sheet having a thickness of 2 mm and having a composition containing C: 0.041%, Si: 3.05%, Mn: 0.081%, S: 0.022% and Te: 0.006% was cold rolled into a thickness of 0.60 mm, and the first cold rolled sheet was intermediately annealed at 900°C for 1 minute and then secondly cold rolled into a final gauge of 0.23 mm. After degreasing, the finally cold rolled sheet was coated with an aqueous dispersion containing 58 mg/I of finely divided Ge and kept at 50°C by means of a pair of fluted rolls. After being left to stand for 8 seconds, the coated steel sheet was passed through a pair of rubber squeeze rollers and then dried. The above treated steel sheet was subjected to a decarburization annealing in wet hydrogen with a heat cycle consisting of a heating at 580°C for 3 minutes and a heating at 850°C for 3 minutes. The decarburized steel sheet was coated with an MgO slurry, dried and then subjected to a final annealing at 870°C for 25 hours under an Ar atmosphere and successively at 1,200°C for 10 hours under an H₂ atmosphere.

The following Table 10 shows the magnetic properties and grain size of the resulting grain-oriented silicon steel sheet together with a comparative grain-oriented silicon steel sheet produced by a conventional method.

It can be seen from Table 10 that a product steel sheet not only having high magnetic induction but also having very low iron loss can be obtained by applying a Ge-containing substance to a finally cold rolled and degreased steel sheet before its decarburization annealing.

### Example 10

A hot rolled sheet having a thickness of 3.0 mm and having a composition containing C: 0.047%, Si: 3.38%, Mn: 0.089%, Se: 0.027% and Sb: 0.026% was annealed at 920°C for 3 minutes and then cold rolled into a thickness of 1.0 mm, and the first cold rolled sheet was intermediately annealed at 950°C for 2 minutes and then secondly cold rolled into a final gauge of 0.30 mm. After degreasing, the finally cold rolled sheet was subjected to a decarburization annealing at 830°C for 3 minutes under an atmosphere consisting of 50% by volume of H₂ and the remainder being N₂ and having a dew point of 60°C. The decarburized steel sheet was coated with an aqueous dispersion containing 200 mg/l of Ge0₂ and kept at 35°C by means of a pair of fluted rolls. After being left to stand for 5 seconds, the coated steel sheet was passed through a pair of rubber squeeze rollers, and then dried in an air bath kept at 180°C. The above treated steel sheet was coated with an MgO slurry, dried and then subjected to a final annealing at 870°C for 30 hours under an Ar atmosphere and successively at 1,200°C for 10 hours under an H₂ atmosphere.

The following Table 11 shows the magnetic properties of the resulting grain-oriented silicon steel sheet together with those of a comparative grain-oriented silicon steel sheet produced by a conventional method.

It can be seen from Table 11 that, when Ge0₂ is applied to the surfaces of a decarburized steel sheet, the resulting product steel sheet has very small crystal grain size and further remarkably excellent magnetic properties.

### Example 11

A hot rolled sheet having a thickness of 2 mm and having a composition containing C: 0.051 %, Si: 3.33%, Mn: 0.069%, Se: 0.027% and Te: 0.007% .was annealed at 1,000°C for 1 minute, and then cold rolled into a thickness of 0.60 mm, and the first cold rolled sheet was intermediately annealed at 950°C for 1 minute and then secondly cold rolled into a final gauge of 0.23 mm. The finally cold rolled sheet was subjected to a decarburization annealing at 835°C for 3 minutes under an atmosphere consisting of 50% by volume of H₂ and the remainder being N₂ and having a dew point of 60°C. The decarburized steel sheet was immersed for 9 seconds in an aqueous dispersion containing 200 mg/l of SnO₂ and kept at 30°C, and then passed through a pair of rubber squeeze rollers, and further dried in an air bath kept at 200°C. The amount of Sn applied to the steel sheet surfaces was 3 mg/m². The above treated steel sheet was applied with an MgO slurry, and then subjected to a final annealing at 870°C for 25 hours under an N₂ atmosphere and successively at 1,200°C for 10 hours under an H₂ atmosphere.

The following Table 12 shows the magnetic properties and grain size of the resulting grain-oriented silicon steel sheet together with those of a comparative grain-oriented silicon steel sheet produced without the application of Sn0₂ according to a conventional method.

It can be seen from Table 12 that an application treatment of an Sn compound to the decarburized steel sheet results in a product steel sheet having very small grain size and remarkably low iron loss.

### Example 12

A hot rolled sheet having a thickness of 3.0 mm and having a composition containing C; 0.048%, Si: 3.28%, Mn: 0.088%, S: 0.025% and Te: 0.008% was annealed at 900°C for 3 minutes and then cold rolled into a thickness of 1.0 mm, and the first cold rolled sheet was intermediately annealed at 950°C for 3 minutes and then secondly cold rolled into a final gauge of 0.30 mm. After degreasing, the finally cold rolled sheet was subjected to a decarburization annealing at 830°C for 3 minutes under an atmosphere consisting of 50% by volume of H₂ and the remainder being N₂ and having a dew point of 60°C. The decarburized steel sheet was immersed for 18 seconds in an aqueous dispersion containing 220 mg/I of As₂S₃ and kept at 40°C, and then passed through a pair of rubber squeeze rollers, and further dried in an air bath kept at 200°C. The amount of As applied to the steel sheet surfaces was 1.4 g/m². Then, the above treated steel sheet was coated with an MgO slurry, dried, and then subjected to a final annealing at 865°C for 30 hours under an N₂ atmosphere and successively at 1,200°C for 10 hours under an H₂ atmosphere.

The following Table 13 shows the magnetic properties and grain size of the product steel sheet together with those of a comparative product steel sheet produced by a conventional method, and illustrates that the present invention is remarkably effective.

### Example 13

A hot rolled sheet having a thickness of 2.0 mm and having a composition containing C: 0.040%, Si: 3.35%, Mn: 0.068%, Se: 0.022% and Sb: 0.029% was annealed at 1,000°C for 1 minute, and then cold rolled into a thickness of 0.60 mm, and the first cold rolled sheet was intermediately annealed at 950°C for 1 minute and then secondly cold rolled into a final gauge of 0.23 mm. The finally cold rolled sheet was subjected to a decarburization annealing at 840°C for 3 minutes under an atmosphere consisting of 50% by volume of H₂ and the remainder being N₂ and having a dew point of 60°C. The decarburized steel sheet was immersed for 30 seconds in an aqueous dispersion containing 400 mg/l of Bi₂0₃ and kept at 80°C, and then passed through rubber squeeze rollers, and further dried in an air bath kept at 150°C. The amount of Bi applied to the steel sheet surfaces was 2.5 mg/m². The above treated steel sheet was coated with an MgO slurry, and then subjected to a final annealing at 870°C for 30 hours -under an N₂ atmosphere and successively at 1,200°C for 10 hours under an H₂ atmosphere.

The following Table 14 shows the magnetic properties and grain size of the resulting product steel sheet together with those of a comparative product steel sheet produced without the application of Bi₂0₃ according to a conventional method.

It can be seen from Table 14 that the application of a Bi salt to a decarburized steel sheet results in a product steel sheet having very small crystal grain size and remarkably low iron loss.

### Example 14

A hot rolled sheet having a thickness of 3.0 mm and having a composition containing C: 0.047%, Si: 3.28%, Mn: 0.089%, S: 0.021 % and Te: 0.006% was annealed at 900°C for 3 minutes and then cold rolled into a thickness of 1.0 mm, and the first cold rolled sheet was intermediately annealed at 950°C for 3 minutes and then secondly cold rolled into a final gauge of 0.30 mm. After degreasing, the finally cold rolled sheet was subjected to a decarburization annealing at 830°C for 3 minutes under an atmosphere consisting of 50% by volume of H₂ and remainder being N₂ and having a dew point of 60°C. The decarburized steel sheet was immersed for 10 seconds in an aqueous solution containing 80 mg/I of ZnS0₄ and kept at 80°C, and then passed through a pair of rubber squeeze rollers, and further dried in an air bath kept at 150°C. The amount of Zn applied to the steel sheet surfaces was 0.75 mg/m². The above treated steel sheet was coated with an MgO slurry, dried, and then subjected to a final annealing under an H₂ atmosphere, wherein the steel sheet was gradually heated at a heating rate of 2.5°C/hr from 800°C to 900°C and successively kept at 1,200°C for 10 hours.

The following Table 15 shows the magnetic properties and grain size of the resulting product steel sheet together with those of a comparative product steel sheet produced by a conventional method.

It can be seen from Table 15 that, when a Zn-containing compound is applied to a decarburized steel sheet, the resulting product steel sheet has very small grain size and further has remarkably low iron loss.

### Example 15

A hot rolled sheet having a thickness of 2.0 mm and having a composition containing C: 0.041 %, Si: 3.29%, Mn: 0.085%, Se: 0.026% andS: 0.029% was annealed at 1,000°C for 1 minute, and then pickled. The pickled sheet was cold rolled into a thickness of 0.60 mm, and the first cold rolled sheet was intermediately annealed at 950°C for 1 minute and then secondly cold rolled into a final gauge of 0.23 mm. The finally cold rolled sheet was subjected to a decarburization annealing at 840°C for 3 minutes under an atmosphere consisting of 50% by volume of H₂ and the remainder being N₂ and having a dew point of 60°C. After an MgO slurry containing 1.5%, calculated as Bi, of Bi₂0₃ was coated onto the surfaces of the decarburized steel sheet, the steel sheet was subjected to a final annealing at 870°C for 30 hours under an N₂ atmosphere and successively at 1,200°C for 10 hours under an H₂ atmosphere.

The following Table 16 shows the magnetic properties, that is, the iron loss W_{17/50} and the magnetic induction Bₗₒ, of the resulting grain-oriented silicon steel sheet together with those of a comparative grain-oriented silicon steel sheet produced by using an MgO slurry containing no Bi₂0₃ according to a conventional method.

It can be seen from Table 16 that the application of an annealing separator containing Bi₂0₃ onto the decarburized steel sheet surfaces is very effective for lowering the iron loss and improving the magnetic induction of the product steel sheet.

According to the present invention, the crystal grain size of the resulting grain-oriented silicon steel sheet can be effectively made into small size, and a grain-oriented silicon steel sheet having high magnetic induction and low iron loss can be obtained.

## Claims

1. A method for producing grain-oriented silicon steel sheets, wherein a hot rolled silicon steel sheet containing at least one of S, Se and Te as an inhibitor for the growth of primary recrystallization grains is subjected to at least one stage cold rolling, the finally cold rolled steel sheet is subjected to a decarburization annealing, and the decarburized steel sheet is coated with an annealing separator consisting mainly of MgO and then subjected to a final annealing, characterised in that at least one member, selected from the group consisting of the elements Ge, Sn, Pb, As, Bi and Zn and compounds containing these elements, is uniformly applied to the surfaces of the finally cold rolled steel sheet before the decarburization annealing.

2. A method according to claim 1 wherein at least one member selected from the group consisting of elements of Ge, Sn, Pb, As, Bi and Zn and compounds containing these elements is uniformly applied to the surfaces of the decarburized steel sheet either additionally or exclusively, prior to the application of the annealing separator to the steel sheet surfaces.

3. A method according to claim 2, wherein the amount of at least one member selected from the group consisting of elements of Ge, Sn, Pb, As, Bi and Zn and compounds containing these elements applied to both surfaces of the steel sheet is at least 10 pg/m² calculated as element.

4. A method for producing grain-oriented silicon steel sheets according to claim 1, wherein the finally cold rolled steel sheet is subjected to a preliminary annealing at a temperature within the range of 500-700°C for 0.5 to 10 minutes, prior to the decarburization annealing.

5. A method according to claim 1 or 4, wherein the amount of at least one member selected from the group consisting of elements of Ge, Sn, Pb, As, Bi and Zn and compounds containing these elements applied to both surfaces of the steel sheet is at least 2 pg/m² calculated as element.

6. A method according to claim 4, wherein the step of applying uniformly at least one member selected from the group consisting of elements of Ge, Sn, Pb, As, Bi and Zn and compounds containing these elements to the surfaces of the steel sheet is carried out before the primary annealing.

7. A method according to claim 4, wherein the step for subjecting the finally cold rolled steel sheet to the preliminary annealing is carried out before the step of applying uniformly at least one member selected from the group consisting of elements of Ge, Sn, Pb, As, Bi and Zn and compounds containing these elements to the surfaces of the steel sheet.

8. A method according to claim 4, wherein the step of applying uniformly at least one member selected from the group consisting of elements of Ge, Sn, Pb, As, Bi and Zn and compounds containing these elements to the surfaces of the finally cold rolled steel sheet is carried out before and after the preliminary annealing.

9. A method for producing grain-oriented silicon steel sheets, wherein a hot rolled silicon steel sheet containing at least one of S, Se and Te as an inhibitor for the growth of primary recrystallization grains is subjected to at least one stage cold rolling, the finally cold rolled steel sheet is subjected to a decarburization annealing, and the decarburized steel sheet is coated with an annealing separator consisting mainly of MgO and then subjected to a final annealing, characterised in that said annealing separator further contains at least one of Bi and compounds containing Bi.

10. A method according to claim 9, wherein the annealing separator contains 0.1-5.0% by weight, calculated as Bi, of at least one of Bi and compounds containing Bi.

## Patentansprüche

1. Verfahren zur Herstellung kornorientierter Silizium-stahlbleche, bei dem ein heiß-gewalztes Siliziumstahlblech, das mindestens eines der Elemente S, Se und Te als Wachstumsinhibitor für primäre Rekristallisationskörner enthält, mindestens einem Kaltwalzschritt unterzogen wird, das letztlich kalt-gewalzte Stahlblech einem Entkohlungsglühen ausgesetzt wird und das entkohlte Stahlblech mit einem hauptsächlich aus MgO bestehenden Glühseparator überzogen und danach einem letzten Glühen unterworfen wird, dadurch gekennzeichnet, daß mindestens ein aus der Gruppe der Elemente Ge, Sn, Pb, As, Bi und Zn sowie der diese Elemente enthaltenden Verbindungen ausgewählter Stoff gleichmäßig auf die Oberflächen des letztlich kalt-gewalzten Stahlblechs vor dem Entkohlungsglühen aufgebracht wird.

2. Verfahren nach Anspruch 1, bei dem mindestens ein aus der Gruppe der Elemente Ge, Sn, Pb, As, Bi und Zn sowie der diese Elemente enthaltenden Verbindungen ausgewählter Stoff gleichmäßig auf die Oberflächen des entkohlten Stahlblechs entweder zusätzlich oder ausschließlich vor dem Auftragen des Glühseparators auf die Stahlblechoberflächen aufgebracht wird.

3. Verfahren nach Anspruch 2, bei dem die Menge des mindestens einen aus der Gruppe der Elemente Ge, Sn, Pb, As, Bi und Zn sowie der diese Elemente enthaltenden Verbindungen ausgewählte und auf beiden Oberflächen des Stahlblechs aufgebrachten Stoffes mindestens 10 Ilg/m2, als Element berechnet, beträgt.

4. Verfahren zur Herstellung kornorientierter Siliziumstahlbleche nach Anspruch 1, bei dem das letztlich kalt-gewalzte Stahlblech vor dem Entkohlungsglühen einem Vorglühen bei einer Temperatur im Bereich von 500 bis 700°C für 0,5 bis 10 Minuten unterzogen wird.

5. Verfahren nach Anspruch 1 oder 4, bei dem die Menge des mindestens einen aus der Gruppe der Elemente Ge, Sn, Pb, As, Bi und Zn sowie der diese Elemente enthaltenden Verbindungen ausgewählte, auf beide Oberflächen des Stahlblechs aufgebrachten Stoffes mindestens 2 Ilg/m2, berechnet als Element, beträgt.

6. Verfahren nach Anspruch 4, bei dem der Schritt des gleichmäßigen Aufbringens mindestens eines aus der Gruppe der Elemente Ge, Sn, Pb, As, Bi und Zn sowie der diese Elemente enthaltenden Verbindungen ausgewählten Stoffes auf die Oberflächen des Stahlblechs vor dem Hauptglühen ausgeführt wird.

7. Verfahren nach Anspruch 4, bei dem der Schritt der Vorglüh-Behandlung des letztlich kalt-gewalzten Stahlbleches vor dem Schritt des gleichmäßigen Aufbringens mindestens eines aus der Gruppe der Elemente Ge, Sn, Pb, As, Bi und Zn sowie der diese Elemente enthaltenden Verbindungen ausgewählten Stoffes auf die Oberflächen des Stahlbleches ausgeführt wird.

8. Verfahren nach Anspruch 4, bei dem der Schritt des gleichmäßigen Aufbringens mindestens eines aus der Gruppe der Elemente Ge, Sn, Pb, As, Bi und Zn sowie der diese Elemente enthaltenden Verbindungen ausgewählten Stoffes auf die Oberflächen des letztlich kalt-gewalzten Stahlbleches vor und nach dem Vorglühen ausgeführt wird.

9. Verfahren zur Herstellung kornorientierter Siliziumstahlbleche, bei dem ein heiß-gewalztes Siliziumstahlblech, das mindestens eines der Elemente S, Se und Te als Wachstumsinhibitor für primäre Rekristallisationskörner enthält, mindestens einem Kaltwalzschritt unterzogen wird, das letztlich kalt-gewalzte Stahlblech einem Entkohlungsglühen ausgesetzt wird und das entkohlte Stahlblech mit einem hauptsächlich aus MgO bestehenden Glühseparator überzogen und danach einem letzten Glühen unterworfen wird, dadurch gekennzeichnet, daß der Glühseparator außerdem Bi und/oder mindestens eine Bi enthaltende Verbindung enthält.

10. Verfahren nach Anspruch 9, bei dem der Glühseparator 0,1 bis 5,0 Gew.-% an Bi und/oder mindestens einer Bi enthaltenden Verbindung, berechnet als Bi, enthält.

## Revendications

1. Une méthode de fabrication de feuilles d'acier au silicium à grain orienté, selon laquelle une feuille d'acier au siiicium laminée à chaud contenant au moins un des éléments S, Se et Te en tant qu'inhibiteur pour la croissance de grains de recristallisation primaire, est soumise à au moins un laminage à froid à une phase, la feuille d'acier laminée finie de laminage à froid étant soumise à une opération de recuit de décarbonisation, la feuille d'acier décarbonisée étant ensuite revêtue d'un séparateur de recuit se composant principalement de MgO, puis soumise à une opération de recuit final, la méthode étant caractérisée en ce qu'au moins une ramification, sélectionnée à partir du groupe se composant des éléments Ge, Sn, Pb, As, Bi et Zn, et de combinaisons contenant ces éléments, est appliquée uniformément sur les surfaces de la feuille d'acier laminée finie de laminage à froid avant l'opération de recuit de décarbonisation.

2. Une méthode selon la revendication 1, dans laquelle au moins une ramification sélectionnée à partir du groupe se composant des éléments Ge, Sn, Pb, As, Bi et Zn et de combinaisons contenant ces éléments, est appliquée uniformément sur les surfaces de la feuille d'acier décarbonisée, soit additionnellement, soit exclusivement, avant l'application du séparateur de recuit sur les surfaces de la feuille d'acier.

3. Une méthode selon la revendication 2, dans laquelle la quantité d'au moins une ramification sélectionnée à partir du groupe se composant des éléments Ge, Sn, Pb, As, Bi et Zn, et de combinaisons contenant ces éléments, appliquée sur les deux surfaces de la feuille d'acier, est au minimum de 10 pg/m², calculée sur la base de l'élément.

4. Une méthode de fabrication de feuilles d'acier au silicium à grain orienté selon la revendication 1, dans laquelle la feuille d'acier laminée finie de laminage à froid est soumise à une opération de recuit préliminaire effectuée à une température se situant dans la gamme de 500-700°C, pendant une durée de 0,5 à 10 minutes, avant l'opération de recuit de décarbonisation.

5. Une méthode selon la revendication 1 ou 4, dans laquelle la quantité d'au moins une ramification sélectionnée à partir du groupe se composant d'éléments de Ge, Sn, Pb, As, Bi et de Zn, et de combinaisons contenant ces éléments, appliquée sur les deux surfaces de la feuille d'acier, est au minimum de 2 pg/m2, cette quantité étant calculée sur la base de l'élément.

6. Une méthode selon la revendication 4, dans laquelle la phase d'application uniforme d'au moins une ramification sélectionnée à partir du groupe se composant d'éléments de Ge, Sn, Pb, As, Bi et Zn, et de combinaisons contenant ces éléments, sur les surfaces de la feuille d'acier, a lieu avant l'opération de recuit primaire.

7. Une méthode selon la revendication 4, dans lequelle la phase consistant à soumettre la feuille laminée finie de laminage à froid à l'opération de recuit préliminaire a lieu avant la phase d'application uniforme d'au moins une ramification sélectionnée à partir du groupe se composant d'éléments de Ge, Sn, Pb, As, Bi et Zn, et de combinaisons contenant ces éléments, sur les surfaces de la feuille d'acier.

8. Une méthode selon la revendication 4, dans laquelle la phase d'application uniforme d'au moins une ramification sélectionnée à partir du groupe se composant d'éléments de Ge, Sn, Pb, As, Bi et Zn, et de combinaisons contenant ces éléments, sur les surfaces de la feuille d'acier laminée finie de laminage à froid a lieu avant et après l'opération de recuit préliminaire.

9. Une méthode de fabrication de feuilles d'acier au silicium à grain orienté, dans laquelle une feuille d'acier au silicium laminée à chaud contenant au moins un des éléments S, Se et Te en tant qu'inhibiteur pour la croissance de grains de recristallisation primaire, est soumise à au moins un laminage à froid à une phase, la feuille d'acier laminée finie de laminage à froid étant soumise à une opération de recuit de décarbonisation, et la feuille d'acier décarbonisée étant ensuite revêtue d'un séparateur de recuit se composant principalement de MgO, puis soumise à une opération de recuit final, la méthode étant caractérisée en ce que le dit séparateur de recuit contient en outre au moins un élément de Bi et des combinaisons contenant du Bi.

10. Une méthode selon la revendication 9, dans laquelle le séparateur de recuit contient de 0,1 à 5,0% en poids, calculé sur la base du Bi, d'au moins un élément de Bi et une des combinaisons contenant du Bi.
